

## UNITED STATES PATENT OFFICE

2,388,563

THERMAL TREATMENT FOR ALUMINUM  
BASE ALLOYS

Joseph A. Nock, Jr., Tarentum, and Theodore W.  
Bossert, Carnegie, Pa., assignors to Aluminum  
Company of America, Pittsburgh, Pa., a cor-  
poration of Pennsylvania

No Drawing. Application July 10, 1943,  
Serial No. 494,244

10 Claims. (Cl. 148—21.1)

This invention relates to a thermal treatment for aluminum base alloys and more particularly to a thermal treatment for stabilizing the working characteristics and the tensile properties of certain annealed precipitation hardening aluminum base alloys.

According to the usual practice of fabricating wrought articles of aluminum base alloys by cold working operations, suitable alloy stock which usually has been previously hot worked, and perhaps cold worked, is given a series of reductions in cross sectional area by rolling, forging or the like at a temperature somewhat below the recrystallization temperature of the alloy, whereby the metal becomes progressively harder and consequently more difficult to work. To alleviate this hardened condition and thereby to make the stock satisfactory for further cold working operations, the material is given an annealing treatment, i. e. heated at a temperature high enough and for a time long enough to cause substantially complete recrystallization of the cold worked metal. The alternate cold working operations and annealing treatments are continued until the final cold worked size and shape of the articles are reached. Although in this procedure each cold working operation generally follows the annealing treatment within a relatively short period of time, i. e. within a period of about four or five days following the annealing treatment, this is not always possible nor convenient and the material in the annealed condition may remain at room temperature for long periods of time, sometimes as long as many months.

In the period between the annealing treatment and the next succeeding working operation, the workability as well as the tensile properties of many aluminum base alloys remains substantially unchanged and is satisfactory for further working operations irrespective of the length of this intervening period, but in age hardening aluminum base alloys containing substantial amounts of magnesium and one or more of the elements copper, silicon and zinc, the workability may progressively decrease throughout this period until further working of the alloy without an additional annealing treatment becomes exceedingly difficult, if not impossible. Whether the aluminum alloy containing magnesium and one or more of the elements copper, silicon and zinc will age harden following the annealing treatment depends upon the amount of these age hardening constituents present in the material and also upon the conditions under which a particular lot of material is annealed and thereafter

cooled to room temperature. In other words, if the age hardening constituents are present in amounts greater than those which are soluble at room temperature and if the annealing conditions are such as to cause retention of more of the age hardening constituents in solid solution than are soluble at room temperature, then that material will age harden upon standing at room temperature, resulting in a progressive diminution of the workability of the material. Consequently, if the period for which this material stands at room temperature is more than a few days, it has been necessary heretofore to re-anneal the material before the next working operation to remove the effect of age hardening on the workability of the material. Since an additional annealing treatment increases the cost of production and since the facilities for giving these alloys this additional annealing treatment are not always readily available immediately preceding the working operation, it is desirable to minimize the change in workability and tensile properties occurring in these alloys following the annealing treatment.

25 An object of this invention is to provide a method of assuring relatively high stability in the working characteristics of the aforementioned annealed age hardening aluminum base alloys, however heated and cooled in the annealing procedure. Another object of this invention is to provide a method of lengthening the period during which the aforementioned annealed precipitation hardening aluminum base alloys can be satisfactorily worked on a commercial scale. 30 35 And still another object is to provide a method of assuring relatively high stability in the mechanical properties of these alloys in the annealed condition.

The term "cold worked" as used throughout 40 the specification and appended claims includes all material having cold working strains, however produced, whether the strains are the result of working the material either above, at, or below the recrystallization temperature of the material. The word "annealed" is used to describe the condition of material which has been cold-worked and then heated at a temperature sufficiently high and for a period sufficiently long to relieve substantially all work hardening strains. 45 50 55 The term "age hardening alloy," when employed herein, refers to an alloy containing age hardening constituents in amounts greater than that soluble at room temperature which has been annealed and cooled from the annealing temperature in such manner that it will age harden if left

standing in that condition at room temperature, resulting in an increase in tensile properties and hardness and a decrease in workability. The term "aluminum base alloy" as herein employed refers to alloys containing at least 75 per cent aluminum by weight.

This invention is predicated upon the discovery that the workability and tensile properties of cold worked and annealed aluminum base alloys containing magnesium and at least one of the elements from the group consisting of copper, silicon and zinc, in amounts sufficient to render the alloys age hardenable, can be rendered relatively stable for long periods of time by heating the annealed alloys to a temperature between about 400° and 600° F. and maintaining them at that temperature for a period of time between about 1/2 and 24 hours. The complete thermal treatment necessary to soften cold worked alloys of this type so that they possess good working characteristics and to retain the good working characteristics indefinitely consists in first annealing the alloys at a temperature between about 650° and 800° F. for a sufficient period of time to relieve substantially all work hardening strains, generally for a time between 1 minute and 20 hours, cooling them to a temperature between 400° and 600° F. and holding them at that temperature for 1/2 to 24 hours, and finally cooling in air to room temperature; or cooling them to room temperature at the end of the annealing treatment and thereafter heating them at a temperature between 400° and 600° F. for 1/2 to 24 hours. Our low temperature treatment is preferably given within a short period of time following annealing, but the beneficial effect of the treatment is not materially decreased if the alloy is stored for a considerable length of time before this treatment is applied. The time required to anneal the aluminum base alloys depends somewhat on the process employed. For example, if a large pile of sheet is annealed in an air heated furnace, the annealing time may be as long as 20 hours. If, on the other hand, the metal is heated as a single piece in a salt bath, then as little time as 1 minute is sufficient to soften the material completely. Furthermore, the manner of heating the alloys in the lower temperature treatment has a corresponding effect on the time required to complete the treatment.

Although our treatment is applicable to all annealed age hardening aluminum base alloys containing magnesium and one or more of the elements copper, silicon or zinc in amounts greater than that soluble at room temperature, it is particularly applicable to aluminum base alloys containing about 3 to 10 per cent zinc, 0.75 to 4 per cent magnesium, and 0.05 to 3 per cent copper since they are especially prone to age hardening after being annealed. In addition to these three alloying ingredients, 0.1 to 1.5 per cent manganese may be present either with or without a small amount of one or more of the grain refining elements titanium, vanadium, zirconium, chromium, cobalt, tungsten, columbium, boron, and tantalum. Other groups of alloys to which our treatment is especially applicable are those containing 3 to 5 per cent copper, 0.5 to 2 per cent magnesium and 0.1 to 1.5 per cent manganese, and those containing 0.05 to 1.0 per cent copper, 0.1 to 3 per cent magnesium and 0.01 to 2 per cent silicon. Small amounts of other alloying elements such as the grain refining elements mentioned above may be added to alloys of either

group without modifying the effect of our treatment on the workability and tensile properties.

Our treatment is effective in preventing progressive diminution of workability in any age hardening aluminum base alloy of the above mentioned compositions. The particular method, such as batch or continuous processes, by which the material is annealed has little or no noticeable influence on our treatment subsequently given to the material. The conditions, however, which may occur during any one of the annealing processes, such as the material being cooled rapidly from the annealing temperature, may have considerable influence on the age hardening characteristics of the material and consequently considerable effect on the particular conditions required by our treatment to stabilize the workability of the material.

As an example of the operation of our invention, an alloy containing 5.25 per cent zinc, 2.1 per cent magnesium, 1.5 per cent copper, 0.4 per cent manganese, 0.3 per cent iron, 0.12 per cent titanium, 0.25 per cent silicon, and balance aluminum, was cold rolled to sheet 0.064 inch in thickness and finally annealed at 650° F. Tensile tests were made on four groups of identical specimens from this material, the groups being designated and treated as follows: 1. Tested immediately after annealing; 2. Stored 6 months at room temperature before being tested; 3. Heated shortly after the annealing treatment at 450° F. for 8 hours, cooled to room temperature, and then immediately tested; 4. Heated shortly after the annealing treatment at 450° F. for 8 hours, cooled to room temperature, and then stored for 6 months at room temperature before being tested. The average values of the tensile properties of the respective groups are given in Table I below:

Table I

| Group  | Tensile strength, lbs./sq. in. | Yield strength, lbs./sq. in. | Per cent elongation |
|--------|--------------------------------|------------------------------|---------------------|
| 1..... | 32,860                         | 12,400                       | 21.5                |
| 2..... | 51,640                         | 27,500                       | 17.0                |
| 3..... | 20,010                         | 11,550                       | 21.0                |
| 4..... | 28,850                         | 11,300                       | 20.0                |

From these examples it is apparent that the tensile properties of the specimens in group 2 changed greatly in 6 months, whereas the properties of the specimens in group 4 by the present treatment were rendered relatively stable over the same period of time. The lower values for the specimens in groups 3 and 4 as compared to those of group 1 are not regarded as being significant for annealed material. The relatively low strength values of groups 1, 3 and 4 are indicative of greater workability than for group 2. While a slight change in the tensile properties may occur during the 6 months period in the alloys given our treatment, these changes are not great enough to seriously affect the workability of the alloys. Since the changes in tensile properties noted above, as well as those observed in many other cases, are of a minor order, the stabilizing treatment is considered to substantially prevent change in the tensile properties and workability of alloys of the type herein described.

We claim:

1. A process for stabilizing the workability and tensile properties of age hardening type of aluminum base alloys containing magnesium and at least one of the elements copper, silicon and zinc that have been annealed and cooled under

conditions that have not substantially eliminated the susceptibility of said alloys to age hardening, comprising heating said alloys in the annealed condition at a temperature between about 400° and 600° F. for a period of time between about  $\frac{1}{2}$  and 24 hours and long enough to remove substantially all tendency for the alloys to age harden.

2. A process for stabilizing the workability and tensile properties of aluminum base alloys containing from 3 to 10 per cent zinc, 0.75 to 4 per cent magnesium, 0.05 to 3 per cent copper that have been annealed and cooled under conditions that have not substantially eliminated the susceptibility of said alloys to age hardening, comprising heating said alloys in the annealed condition at a temperature between about 400° and 600° F. for a period of time between  $\frac{1}{2}$  and 24 hours and long enough to remove substantially all tendency for the alloys to age harden, and finally cooling the alloys to room temperature.

3. A process for stabilizing the workability and tensile properties of aluminum base alloys containing from 3 to 5 per cent copper, 0.5 to 2 per cent magnesium and 0.1 to 1.5 per cent manganese that have been annealed and cooled under conditions that have not substantially eliminated the susceptibility of said alloys to age hardening, comprising heating said alloys in the annealed condition at a temperature between about 400° and 600° F. for a period of time between about  $\frac{1}{2}$  and 24 hours and long enough to remove substantially all tendency for the alloys to age harden, and finally cooling the alloys to room temperature.

4. A process for annealing and stabilizing the workability and tensile properties of cold worked aluminum base alloys containing from 3 to 10 per cent zinc, 0.75 to 4 per cent magnesium, 0.05 to 3 per cent copper, comprising annealing said alloys until substantially all work hardening strains are relieved under conditions of annealing and cooling that do not substantially eliminate the susceptibility of said alloys to age hardening, then heating said alloys at a temperature within the range of about 400° to 600° F. for a period of time between  $\frac{1}{2}$  and 24 hours and long enough to remove substantially all tendency for the alloys to age harden.

5. A process for annealing and stabilizing the workability and tensile properties of cold worked aluminum base alloys containing from 3 to 10 per cent zinc, 0.75 to 4 per cent magnesium, 0.05 to 3 per cent copper, comprising annealing said alloys until substantially all work hardening strains are relieved under conditions of annealing and cooling that do not substantially eliminate the susceptibility of said alloys to age hardening, cooling them to room temperature, then heating said alloys at a temperature within the range of about 400° to 600° F. for a period of time between about  $\frac{1}{2}$  and 24 hours and long enough to remove substantially all tendency for the alloys to age harden, and finally cooling the alloys to room temperature.

6. A process for annealing and stabilizing the workability and tensile properties of cold worked aluminum base alloys containing from 3 to 10 per cent zinc, 0.75 to 4 per cent magnesium, 0.05 to 3 per

cent copper, comprising continuously annealing said alloys at a temperature between 650° and 800° F., under conditions of annealing and cooling that do not substantially eliminate the susceptibility of said alloys to age hardening, then heating said alloys at a temperature within the range of about 400° to 600° F. for a period of time between about  $\frac{1}{2}$  and 24 hours and long enough to remove substantially all tendency for the alloys to age harden, and finally cooling the alloys to room temperature.

7. A process for annealing and stabilizing the workability and tensile properties of cold worked aluminum base alloys containing from 3 to 10 per cent zinc, 0.75 to 4 per cent magnesium, 0.05 to 3 per cent copper, comprising annealing said alloys until substantially all work hardening strains are relieved under conditions of annealing and cooling that do not substantially eliminate the susceptibility of said alloys to age hardening, thereupon cooling said alloys to a temperature between about 400° and 600° F., holding them at a temperature within said range of temperatures for a period of time between about  $\frac{1}{2}$  and 24 hours and long enough to remove substantially all tendency for the alloys to age harden, and thereafter cooling the alloys to room temperature.

8. A process for stabilizing the tensile properties of aluminum base alloys containing from 3 to 10 per cent zinc, 0.75 to 4 per cent magnesium, 0.05 to 3 per cent copper that have been annealed and cooled under conditions that have not substantially eliminated the susceptibility of said alloys to age hardening, comprising heating said alloys in the annealed condition at about 450° F. for about 8 hours, and thereafter cooling the alloys to room temperature.

9. A process for annealing and stabilizing the workability and tensile properties of cold worked aluminum base alloys containing magnesium and at least one of the elements copper, silicon and zinc, comprising annealing said alloys until substantially all work hardening strains are relieved under conditions of annealing and cooling that do not substantially eliminate the susceptibility of said alloys to age hardening, then heating said alloys at a temperature within the range of about 400° to 600° F. for a period of time between about  $\frac{1}{2}$  and 24 hours and long enough to remove substantially all tendency for the alloys to age harden.

10. A process for annealing and stabilizing the workability and tensile properties of cold worked aluminum base alloys containing from 3 to 5 per cent copper, 0.5 to 2 per cent magnesium and 0.1 to 1.5 per cent manganese, comprising annealing said alloys until substantially all work hardening strains are relieved under conditions of annealing and cooling that do not substantially eliminate the susceptibility of said alloys to age hardening, then heating said alloys at a temperature within the range of about 400° to 600° F. for a period of time between about  $\frac{1}{2}$  and 24 hours and long enough to remove substantially all tendency for the alloys to age harden.

JOSEPH A. NOCK, JR.  
THEODORE W. BOSSERT.

CERTIFICATE OF CORRECTION.

Patent No. 2,388,563.

November 6, 1945.

JOSEPH A. NOCK, JR., ET AL.

It is hereby certified that error appears in the printed specification of the above numbered patent requiring correction as follows: Page 1, first column, line 9, for the word "within" read --which--; and that the said Letters Patent should be read with this correction therein that the same may conform to the record of the case in the Patent Office.

Signed and sealed this 29th day of January, A. D. 1946.

Leslie Frazer

(Seal)

First Assistant Commissioner of Patents.